

June 17, 1958

H. T. BELLAMY

2,839,292

REFRACTORY RESERVOIR FOR ALUMINUM

Filed Aug. 9, 1954



Inventor  
Harry T. Bellamy  
by Bair, Freeman & Molinare  
Atty's.

1

2,839,292

**REFRACTORY RESERVOIR FOR ALUMINUM**

Harry T. Bellamy, Evanston, Ill.

Application August 9, 1954, Serial No. 448,609

3 Claims. (Cl. 266—34)

2

but so far as I am aware, no one previously appreciated its remarkable resistance to the corrosive action of molten aluminum.

My invention consists in rendering parts or articles that are normally attacked by molten aluminum resistant to such attack by coating the surface thereof with molybdenum or tungsten. Molybdenum may be conveniently applied by well known processes including metallizing (spraying), plating or cladding. I have found that an especially convenient means of applying a uniform continuous molybdenum coating is by spraying. When the part being sprayed is made from a ferrous metal or ferrous alloy, the molybdenum bonds tenaciously to a clean, warm surface. Steel parts have been provided with a wear resistant coating of molybdenum by spraying for some time. When the molybdenum sprayed part is to be subjected to thermal shock, "Inconel," an alloy comprising substantially 80% nickel, 12-14% chromium and 6-8% iron, is preferred as the base metal due to its similar coefficient of expansion.

Most refractory parts associated with an aluminum melting furnace or the like are completely submerged in molten aluminum. However, some parts may become exposed to air at temperatures approaching the temperature prevailing within the furnace as, for example, when the level of the molten aluminum falls below its maximum height. Under such conditions the molybdenum coating will oxidize and lose its refractoriness and corrosion resistance. Therefore, parts subject to oxidation are first coated with molybdenum and then given an external coating of a suitable refractory material that will protect the metallic coating from oxidation, such as a conventional ceramic coating composition, or a molybdenum alloy containing a minor proportion of chromium and/or nickel. Ceramic compositions can be applied by dip coating or spraying an aqueous solution or suspension thereof, or they may be applied by what is known as "flame spraying." This process involves the use of a "gun" equipped with a hot gas flame through which the powdered ceramic material is blown, thus converting the solid powder into fused flaming particles which deposit on the part and solidify as a firmly adhering coating. A ceramic coating thus applied does not provide an impervious film over the entire surface, and if it were used without an intermediate molybdenum film the part would corrode, the molten aluminum attacking rapidly through the imperfections in the surface coating. The ceramic coating will provide protection for molybdenum against oxygen in areas which become exposed to air upon removal from molten aluminum. In areas where the ceramic coating may fail, the extent of the oxidation is not sufficient to permit any substantial attack by the aluminum because the oxidized areas are small and the exposure to aluminum is not continuous.

Various examples of my invention are illustrated in the accompanying drawings, in which:

Figure 1 is a vertical section through an electric melting furnace having a connecting tube constructed in accordance with the invention;

Figure 2 is a sectional view taken along the line 2—2 of Figure 1;

Figure 3 is an elevational view, partly in section, of a bubble tube immersed in molten aluminum;

Figure 4 is a plan view of an electrical immersion heater having a coating applied in accordance with the invention; and

Figure 5 is an enlarged cross-sectional view taken along the line 5—5 of Figure 4.

The furnace shown in Figure 1 is of conventional construction and comprises a casing or housing 11 which may be made of metal and which supports a cast ceramic body 16 containing a melting chamber 12 and a holding

This invention relates to refractory articles or parts that are resistant to corrosion by molten aluminum and to a method for making such articles.

At its melting point of 1216° F. or above, aluminum is highly corrosive and rapidly attacks common structural metals. Tubing of iron, ferrous alloys, alloys of chromium, nickel and copper, for example, when dipped into molten aluminum will pit and develop holes completely through the wall thereof within a relatively short time. Attempts to coat or plate these metals and alloys to protect them from this corrosive action have been disappointing. Common plating metals, such as chromium and nickel, are vigorously attacked by molten aluminum. Ceramic compositions, although resistant to molten aluminum, cannot successfully be applied in a continuous film, primarily due to difference in the coefficient of thermal expansion between the ceramic and the metal base. Invariably some surface defect develops, such as pinholes or cracks in the coating, to blemish the continuity of the surface, and attack by the molten aluminum results at these points. Consequently, parts which must be capable of resisting attack by molten aluminum are conventionally made from cast or otherwise shaped solid ceramic compositions. Pyrometer protecting tubes, for example, are formed by extruding a refractory ceramic which contains a high proportion of silicon carbide with a suitable bonding material.

Other parts adapted to resist molten aluminum are made from graphite. Both graphite and the ceramic parts stand up fairly well under the corrosive action of aluminum, but are disadvantageous in that they are brittle and break very easily during installation or other handling. Graphite has the additional disadvantage of quickly oxidizing at elevated temperatures. These non-metallic parts are also rather difficult and expensive to fabricate as compared with ferrous metals, for example. The aluminum casting industry has been in need of a suitable material that will withstand molten aluminum and which at the same time does not have the shortcomings of the brittle non-metallic parts now commonly used.

I have discovered that molybdenum and tungsten offer surprising resistance to corrosion by molten aluminum and that these metals serve admirably as a coating for materials that are normally subject to attack by molten aluminum. These metals are highly refractory, molybdenum having a melting point of 4750° F., and tungsten having a melting point of 6170° F. That molybdenum and tungsten should be capable of resisting attack by molten aluminum was especially surprising in view of the fact that chromium, which is also in group VI of the periodic table, and would predictably react chemically in the same manner as molybdenum and tungsten, is vigorously disintegrated by molten aluminum.

Of the two operable metals, molybdenum is the most readily available and the easier to fabricate, and it is, therefore, preferred over tungsten. Molybdenum has been known and commercially available for many years,

chamber 14 interconnected by means of horizontally-spaced channels or tubes 18. A magnetic core 15 is arranged around the tubes and is energized by alternating current windings (not shown) to induce a melting current in the aluminum metal within the tubes. Since all of the melting occurs within the tubes, the prevailing current density is very high and, consequently, this portion of the furnace deteriorates much more rapidly than the melting and holding chambers. The improvement in the construction illustrated lies in the tube 18, which is made from molybdenum metal.

One method of incorporating the molybdenum tube 18 into the furnace is to support it by a refractory block 20, which is cast around the tube. The supporting block 20 may be conveniently made from a mixture similar to the ceramic composition 16, which consists of Lumnit cement (commercial heat-resistant hydraulic cement) and a suitable aggregate. If the enclosed tube is prepared separately in this way, the bond to the ceramic mass may be more carefully controlled.

Another method, however, consists in casting the ceramic composition 16 around the tube 18 simultaneously with the formation of the melting and holding chambers.

The molybdenum tube will outlast the conventional ceramic tube many times, and, of course, is not subject to breakage. To insure against oxidation of the molybdenum tube, it is preferred that the molybdenum tube be coated inside and out prior to enclosure in cast composition 16, or in the block 20, with a suitable oxidation protective coating that will withstand temperatures in the vicinity of 1500° F., and which preferably will also resist molten aluminum. A vapor-phase deposited silicon coating or other ceramic coating, such as magnesium or calcium oxides, are suitable for this purpose. In an installation of this kind the primary source of oxygen is due to permeation of air through the ceramic composition 16. The oxidation that might occur would not be severe, but it is preferable to protect against it in the manner described.

Figure 3 shows a bubble tube which is commonly used in aluminum foundries to introduce gases, such as nitrogen or chlorine, into molten aluminum. The conventional tube is made from graphite and deteriorates rather rapidly due to oxidation and, of course, such tubes are highly brittle and are frequently broken.

The bubble tube 35 of Figure 3 has been made in accordance with the invention and consists of a standard length of suitable diameter standard iron pipe 32 threaded at one end and closed at the other. The closed lower end contains a suitable number of holes 36 for permitting the escape of gas through the wall of the tube. The surface of the metal is cleaned thoroughly to remove any dirt or grease and a coating 33 of molybdenum, about .005 inch thick or more, is sprayed over the surface. To protect the molybdenum coating 33 from oxidation a ceramic coating 34 is applied thereover by flame spraying or by applying a coating by other means. The standard ferrous metal base coated in this manner is practically unbreakable since the layers are securely bonded together. It will resist attack by molten aluminum almost indefinitely. In use, the tube 35 is connected to the gas line 37 through an elbow 38, and dips into molten aluminum 31 in the refractory container 30.

Figures 4 and 5 illustrate an electrical immersion heater 40 of conventional construction, which has been treated according to the invention. The heater contains the usual electrical resistor core 44 sheathed in an insulating material 45 and an external metal housing 46 which is normally subject to corrosion by molten aluminum. This immersion unit may be protected from the action of molten aluminum in accordance with this invention by first spraying the surface with about .006 to .008 inch of molybdenum 47. The unit may be coated with molybdenum by cladding or electroplating instead of spraying. An oxidation protective ceramic coating then may be applied over the molybdenum coating over any areas not to be covered by molten aluminum. Such an immersion unit has been found to provide very satisfactory service in molten aluminum.

It is also within the scope of the invention to provide parts for pumps and the like, used in contact with molten aluminum, made from molybdenum or tungsten metal.

The invention has been illustrated by way of a number of articles or parts which commonly are used in molten aluminum, but it is not my intention to limit the invention thereto otherwise than as necessitated by the appended claims. Furthermore, various modifications of the invention will become apparent to those skilled in the art without departing from the spirit of the invention.

I claim as my invention:

1. In combination, a refractory reservoir for molten aluminum and a tube disposed therein below the normal level of the molten aluminum, said tube being made from a ferrous metal coated with an intermediate layer of molybdenum and an external layer of ceramic composition whereby said tube is protected from corrosion by molten aluminum and from oxidation.
2. In combination, a refractory reservoir for molten aluminum and a tube disposed therein below the normal level of the molten aluminum, said tube being made from an alloy containing substantially 80% nickel, 12 to 14% chromium and 6 to 8% iron and coated with an intermediate layer of molybdenum and an external layer of ceramic composition whereby said tube is protected from corrosion by molten aluminum and from oxidation.
3. An aluminum melting furnace having two chambers adapted to hold molten aluminum, said chambers being interconnected by a ferrous metal tube having its surface coated with an intermediate layer of molybdenum and an external layer of ceramic composition.

#### References Cited in the file of this patent

#### UNITED STATES PATENTS

|           |                 |               |
|-----------|-----------------|---------------|
| 1,582,407 | King            | Apr. 27, 1926 |
| 2,149,657 | Armstrong       | Mar. 7, 1939  |
| 2,447,672 | Smith et al.    | Aug. 24, 1948 |
| 2,508,465 | Offinger et al. | May 23, 1950  |
| 2,508,466 | Brace           | May 23, 1950  |
| 2,588,421 | Shepard         | Mar. 11, 1952 |
| 2,648,715 | Lillienberg     | Aug. 11, 1953 |
| 2,650,903 | Garrison et al. | Sept. 1, 1953 |
| 2,665,474 | Beidler et al.  | Jan. 12, 1954 |

#### OTHER REFERENCES

Metals Handbook. 1948 edition, published by The American Society of Metals (pages 1057-1058 relied on).